

# UNITED STATES PATENT OFFICE.

CHESNEY L. JONES, OF OAKLAND, NEW JERSEY, ASSIGNOR OF ONE-HALF TO FRED J. MOLT, OF RIVERDALE, NEW JERSEY.

## COMPOSITION OF MATTER.

1,244,742.

Specification of Letters Patent. Patented Oct. 30, 1917.

No Drawing.

Application filed February 8, 1917. Serial No. 147,280.

To all whom it may concern:

Be it known that I, CHESNEY L. JONES, a citizen of the United States, and residing at Oakland, in the county of Bergen and 5 State of New Jersey, have invented a certain new and useful Composition of Matter, of which the following is a specification, such as will enable those skilled in the art to which it appertains to make and use the 10 same.

The object of my invention is the production of a composition metal which has the appearance of silver and the strength of steel but which will not rust by exposure to 15 the atmosphere or to anything else which ordinarily causes metals to corrode; a further object being to produce a metal which will resist most acids and which will take a high polish, can be cast or rolled into bars 20 or sheets, or forged or otherwise fashioned into desired forms, and which is very tough and from which springs and like articles may also be formed.

My composition consists of the following 25 ingredients combined in the manner set out.

|           |        |
|-----------|--------|
| Nickel    | 67.8%  |
| Copper    | 28.0%  |
| Manganese | 02.5%  |
| Iron      | 01.5%  |
| Vanadium  | 00.2%  |
|           | 100.0% |

In the practice of my invention the nickel, 35 copper, manganese and iron are preferably first melted in any suitable furnace or crucible, and the vanadium is mingled therewith after the other metals have been melted and drawn into the ladle or in cases where crucibles are employed or used for melting, just 40 before the metal is to be poured, or in other words, as soon as the melting product is taken from the furnace, and the product thus formed is thoroughly stirred and the 45 various component parts mingled.

It is possible, however, to mingle all the component parts, including the vanadium,

and then melt the product, but the process of procedure first above named is the one preferred.

50

The vanadium adds considerable to the strength and toughness of the finished metal and the amount of vanadium can be varied slightly, but should preferably never be over 1% of the total mixture, and when the 55 amount of vanadium employed varies from the figures given in the formula, the amount of copper should also be varied to an equal extent.

I may also add carbon to the above ingredients, to the extent of from .18 to .20%, 60 and this will make the metal product harder, the temper depending on the percentage of carbon employed.

My invention is not limited to the exact 65 proportions of the various ingredients thereof, as herein set out, and changes therein and modifications thereof may be made, within considerable limits, without departing from the spirit of the invention or sacrificing its 70 advantages.

Having fully described my invention, what I claim as new and desire to secure by Letters Patent, is:—

1. The composition metal herein described 75 containing nickel, copper, manganese, iron and vanadium.

2. A metallic compound comprising, 80 nickel, copper, manganese, iron, vanadium and carbon, combined.

3. The composition metal herein described 85 consisting of nickel 67.8%, copper 28.0%, manganese 2.5%, iron 1.5% and vanadium .2%, said ingredients being combined substantially as described.

In testimony that I claim the foregoing as my invention I have signed my name in presence of the subscribing witnesses this 7th day of February 1917.

CHESNEY L. JONES.

Witnesses:

C. E. MULREANY,  
H. E. THOMPSON.